

## UNITED STATES PATENT OFFICE

2,140,905

## TURBINE BLADE

Russell Franks, Niagara Falls, N. Y., assignor to  
Union Carbide and Carbon Research Laboratories, Inc., a corporation of New York

No Drawing. Application May 2, 1936,  
Serial No. 77,549

2 Claims. (Cl. 253—77)

This invention relates to improved high-chromium alloy steel turbine blades for use at elevated temperatures.

It is important that the blades employed in turbines possess high strength and appreciable ductility and toughness when exposed to superheated steam at high pressures. In addition to these special engineering characteristics the steel must retain satisfactory strength and ductility for a reasonable length of time at the operating temperature, and must offer considerable resistance

to corrosion, without decreasing undesirably the ductility of the material.

The effect of nitrogen in increasing the hardenability of the high chromium steels without seriously decreasing their ductility or toughness is clearly illustrated by the following table of data representing the physical properties of several steels containing about 13% chromium, about 0.07% carbon, small fractional amounts of silicon and manganese; and the amounts of nitrogen indicated in the first column:

| Percent N | Condition of metal* | Yield pt. lb./sq. in. | Maximum stress lb./sq. in. | Percent elongation in 2" | Percent Red. of area | Izod impact ft. lb. | Brinell hardness |
|-----------|---------------------|-----------------------|----------------------------|--------------------------|----------------------|---------------------|------------------|
| 0.025     | 1                   | 139,000               | 151,000                    | 10                       | 15                   | 5                   | 293              |
| 0.025     | 2                   | 66,000                | 95,500                     | 23                       | 60                   | 58                  | 187              |
| 0.025     | 3                   | 44,000                | 78,500                     | 30                       | 71                   | 101                 | 137              |
| 0.08      | 1                   | 178,000               | 194,000                    | 5                        | 11                   | 4                   | 402              |
| 0.08      | 2                   | 108,500               | 123,500                    | 21                       | 65                   | 60                  | 228              |
| 0.08      | 3                   | 66,500                | 90,500                     | 26                       | 66                   | 100                 | 179              |

\* 1=Oil quenched from 950° C.

2=Oil quenched from 950° C., then held 2 hours at 600° C. and air cooled.

3=Held 3 hours at 750° C. and air cooled.

25 to the oxidation that normally occurs at elevated temperatures.

In the early attempts to employ high chromium steels for this purpose, it was found that the chromium content must be closely controlled if the desired physical characteristics were to be attained. If the chromium content is too low, the strength of the steel is too low and the steel does not offer sufficient resistance to oxidation. On the other hand, if the chromium is too high, the steel cannot be given satisfactorily high strength, without at the same time rendering it excessively brittle. Thus, it was found necessary to employ a steel containing between about 11% and about 14% chromium. Even in steels of this type difficulty has been met in securing the desired strength without producing an undesirable brittleness. Some improvement has been secured by introducing small amounts of certain hardening elements, such as nickel, copper, tungsten, and molybdenum.

I have found that certain chromium steels containing nitrogen perform unusually well as turbine blades. Although the usefulness of this discovery is not limited to or by any theory, it is believed that the presence of chromium nitrides, which have a high solubility in the chromium iron solid solutions, greatly increases the hardening capacity of the steels, and it imparts improved hardenability without rendering the metal excessively brittle or of inferior ductility. Furthermore, when nitrogen is present in the steels, it is possible to increase the chromium content and thereby secure a greater resistance to cor-

rosion, without decreasing undesirably the ductility of the material.

The effect of nitrogen in increasing the hardenability of the high chromium steels without seriously decreasing their ductility or toughness is clearly illustrated by the following table of data representing the physical properties of several steels containing about 13% chromium, about 0.07% carbon, small fractional amounts of silicon and manganese; and the amounts of nitrogen indicated in the first column:

According to the present invention turbine blades comprise steels having a chromium content between about 12% and 16%, carbon in amounts up to about 0.20%, about 0.05% to 0.20% nitrogen, and the remainder iron, except for the customary small amounts of impurities and alloyed additions made to ordinary steels of similar chromium content. Preferably, neither the nitrogen content nor the carbon content exceeds about 0.12% of the steel.

I claim:

1. Turbine blade having high strength, high resistance to oxidation, and high ductility and toughness when exposed to superheated steam at high pressures, said turbine blade being composed of a steel containing about 12% to about 16% chromium, carbon in amounts up to about 0.2%, and about 0.05% to less than 0.2% nitrogen, the remainder being substantially all iron, the nitrogen being distributed substantially uniformly throughout the steel.

2. Turbine blade for use at high temperatures and having high strength, high resistance to oxidation, and high ductility and toughness when exposed to superheated steam at high pressures, said turbine blade being composed of a steel containing about 12% to 16% chromium, carbon in amounts not exceeding about 0.12%, and about 0.05% to 0.12% nitrogen, the remainder being substantially all iron the nitrogen being distributed substantially uniformly throughout the steel.

RUSSELL FRANKS.